

# UNITED STATES PATENT OFFICE.

JACOB OLTMANS, OF HILVERSUM, NETHERLANDS.

## PROCESS FOR THE MANUFACTURE OF PLIANT FLOOR-COVERING.

1,356,784.

Specification of Letters Patent. Patented Oct. 26, 1920.

No Drawing.

Application filed February 7, 1919. Serial No. 275,651.

To all whom it may concern:

Be it known that I, JACOB OLTMANS, a subject of the Queen of the Netherlands, and residing at 60 Loosdrechtsczeweg, Hilversum, the Netherlands, have invented certain new and useful Improvements in Processes for the Manufacture of Pliant Floor-Covering, of which the following is a specification.

10 This invention relates to a process for the manufacture of a pliant floor covering.

It is well-known that hitherto for the covering of floors the so-called linoleum is generally used which is a composition made out 15 of a mixture of linseed oil contingently partly oxidized, with filling materials such as wood flour and cork powder, the said mixture being applied for coating a fabric or tissue generally consisting of jute.

20 As the linseed oil oxidizes when exposed to the air the at first wet, plastic material obtains the dryness and solidity required for its use as a floor covering.

The oxidation process requires rather a 25 long time; as a consequence thereof the linoleum is only ready for use about one year after its manufacture.

Owing to this fact the storing of large 30 quantities of linoleum is necessary so that the cost price of the article is considerably increased.

Moreover it is necessary to apply a first 35 layer of jute fabric because the plastic mass is but little coherent the stickiness of the mass being diminished by adding a large quantity of clay and chalk. The application of said layer makes the linoleum a very costly product especially as the jute prices are very high.

40 The floor covering according to the present invention differs from the linoleum inasmuch no oil is used and no backing of jute or the like is employed.

In the method according to the invention 45 glue is used as a binding agent. It has appeared that with the aid of this binding agent it is possible to make a floor covering without a backing.

The economical advantages of this are 50 quite obvious.

As the glue dries quickly the product may be used a few days after it has been prepared. So in the works which produce the floor covering according to the invention a 55 commercial product is obtained which may be transported immediately, whereas the

usual linoleum should be stored during a long time before it has the properties commercially required.

Moreover the glue is much cheaper than 60 oil and the expensive jute fabric is not required.

The invention mainly consists in the way in which the glue is added to and mixed with the filling material and further consists 65 in the proportions of the raw materials and the combination of the said materials.

The proportions are very important to obtain a thick plastic mass which may be rolled 70 and which solidifies at normal temperature.

The other features of the invention may be suitably set forth by an example as follows:

It is of course evident that in many respects this process may be varied without departing from the spirit and scope of the invention.

In order to make a sheet of floor covering which may be rolled up that has a length 75 of 3 feet and usual breadth of 6 feet one may proceed as follows:

A quantity of 1500 grams filling material such as wood flour or cork powder is saturated with a dilute solution of glue of about 1:10 until the mass has obtained a weight 80 of 3500 grams. This saturation has for its object to prevent the binding mass from being absorbed by the wood or cork flour after the former has been added. Preferably a coloring substance is previously added to the glue solution so that the wood flour or cork powder obtains the required color.

85 800 grams of glue dissolved in 2400 grams of water are subsequently added. To this solution 150 grams of nitric acid are added to increase the adhesive properties of the glue. The nitric acid causes the wood or cork powder to dissolve more or less and to make it pappy or pulpy.

90 Another advantage is that the glue remains liquid which is important for the further treatment especially for the rolling of the mass. Finally the addition of nitric acid prevents the mass from drying too soon 95 which would cause the bulging and warping of the sheet, whereas according to the invention smooth and equal sheets are produced.

To further increase the stickiness of the 100 glue 300 grams of sugar are added to the mass. By this addition the product remains pliant, whereas moreover a fermentation

sets in that renders the mass somewhat porous and gives it the appearance of rubber.

The subsequent addition of 600 grams of glycerin has for its object to produce the required suppleness; to make the color clear and fresh 300 grams of alum solution are added.

Finally the mass is mixed with 640 grams of china-clay, lenswhite, magnesia or another filling material containing little or 10 no lime. By mixing the above substances thoroughly with the aid of appropriate machinery a homogeneous mass is obtained which is then rolled to sheets of the required thickness.

15 As no use is made of jute or another fabric it is desirable to strengthen the mass during the treatment. This may be attained by applying a piece of fabric of the required dimensions on which the mass is

20 spread out and passed together through the rollers. When the sheets are ready, they are put into a drying room in order to obtain the properties required.

To make the material insoluble in water 25 and to obtain the required hardening, after some days the sheets may be spread over with formalin, while the fabric which has served as a support may be removed after some days. The pliant floor covering obtained in this way possesses notwithstanding the lack of a fabric or even of a fibrous material an extraordinary resistance which must be ascribed to the toughness of the applied glue.

30 In order to make the glue insoluble in water at the beginning of the process one may also add to the glue solution chromates or other substances which have the property to coagulate glue and to render it insoluble.

40 The product according to the invention after having been kept some days in the drying room may be rolled together and is ready for use.

Having now described my invention, what

I claim as new and desire to secure by Letters Patent is:

1. In a process for preparing a pliant floor covering comprising a filling material and a binding mass composed of a heavy glue and a dilute glue solution, the step of 50 treating the filling material with the dilute glue solution previous to the mixing with the heavy glue.

2. In a process for preparing a pliant floor covering comprising a filling material 55 and a binding mass, composed of a heavy glue and a dilute glue solution, the step of treating the filling material with the dilute glue solution previous to the mixing with the heavy glue, in connection with the step of 60 adding nitric acid to the binding mass and incorporating the mass with the heavy glue, after the latter has been treated with nitric acid.

3. In a process for preparing a pliant 65 floor covering composed of a filling material and a binding mass, including a solution of dilute glue and a heavy glue, the step of saturating the filling material with a quantity of the dilute glue solution, mixing the 70 material with the binding mass and coagulating an additional quantity of glue solution.

4. A pliant floor covering containing the 75 reaction products of glue, glycerin, a coagulating agent, nitric acid and wood flour.

5. A pliant floor covering containing the reaction products of glue, glycerin, a coagulating agent, nitric acid and wood flour and a filling material.

6. A pliant floor covering containing the reaction products of about 110-120 parts of glue, 60 parts of glycerin, a coagulating agent, 15 parts of nitric acid and 150 parts of wood flour, and a filling material.

85 In testimony whereof I affix my signature.

JACOB OLTMANS.